

# UNITED STATES PATENT OFFICE.

ADOLF WINTHER, AUGUST LEOPOLD LASKA, ARTHUR ZITSCHER, FELIX KUNERT, AND EDWIN ACKER, OF OFFENBACH-ON-THE-MAIN, GERMANY, ASSIGNEES TO CHEMISCHE FABRIK GRIESHEIM-ELEKTRON, OF FRANKFORT-ON-THE-MAIN, GERMANY, A CORPORATION.

## PRODUCING ICE COLORS.

1,099,108.

Specification of Letters Patent.

Patented June 2, 1914.

No Drawing.

Application filed October 16, 1913. Serial No. 795,456.

To all whom it may concern:

Be it known that we, ADOLF WINTHER, AUGUST LEOPOLD LASKA, ARTHUR ZITSCHER, FELIX KUNERT, and EDWIN ACKER, citizens 5 of the German Empire, and residents of Offenbach-on-the-Main, in the Grand Duchy of Hesse, Germany, with the post-office addresses Mainstrasse 159, Wilhelmsplatz 18, Friedrichstrasse 31, Sennefelderstrasse 77, 10 and Krafftstrasse 14, respectively, have invented new and useful Improvements in Producing Ice Colors, of which the following is a specification.

Our invention relates to an improvement 15 in the art of producing ice-colors, that is producing dyes by combining the components directly on the vegetable fiber, consisting in treating cotton goods, which have been impregnated with a solution of an arylamid of 20 2,3-oxynaphthoic acid, but have not been dried, with a nonsulfonated diazo compound. Under the term cotton goods we include cotton yarn, cops, cross-reels and loose cotton.

The success of the present invention could 25 not be foreseen from the antecedent publications, because cotton goods, which have been impregnated with beta-naphthol, must be dried before the development with diazo compounds. The cotton yarn or loose cotton 30 ton goods, which has been impregnated with a solution of an arylamid of 2,3-oxynaphthoic acid, yields, however, as contrasted with beta-naphthol equal, powerful and useful shades also, when developed with diazo 35 compounds, while wet.

As arylamids of 2,3-oxynaphthoic acid there can be employed the anilid of 2,3-oxynaphthoic acid itself, its substitution products, which are formed by substituting anilin 40 by its substitution products, such as for example its homologues and chloro- and nitro-substitution products for the condensation with 2,3-oxynaphthoic acid and also the substitution products, which are obtained by 45 condensing two molecular proportions of 2,3-oxynaphthoic acid with one molecular proportion of a diamin, such as for example the condensation products from 2,3-oxynaphthoic acid and phenylen-diamin, tolulylene-diamin, benzidin and so on. As diazo 50 compounds all can be employed not containing a sulfo group, such as for example the diazo compounds derived from anilin and

its substitution products, from anisidin, from amidoazo compounds, alpha- and beta-naphthylamin, benzidin, tolidin, dianisidin and from other diamidobases.

Therefore not only the dyestuffs, described in U. S. Patents Nos. 1034853 and 1042356, can be employed for the present process, but all, which can be formed by combining one of the above mentioned diazo compounds with one of the mentioned arylamids of 2,3-oxynaphthoic acid.

In order to illustrate the new process more fully the following examples are given, the parts being by weight.

*Example I. Production of the dyestuff, obtained by combining diazotized para-nitro-ortho-toluidin with the anilid of 2,3-oxynaphthoic acid, on cotton yarn.*

The completely dried bleached or raw cotton-yarn, previously boiled with carbonate of soda or caustic soda, is impregnated with a hot solution of the anilid of 2,3-oxynaphthoic acid. The yarn is well handled 75 3 or 4 times in an earthen pot, wrung out, handled once more and finally wrung out as well as possible. After the yarn has been beaten in order to secure uniform impregnation and has completely cooled, it is introduced in a wet condition into the dye-bath, well handled, wrung out and allowed to hang for a short time before being passed through the bath a second time, if necessary.

Solutions suitable for use are made as follows:

*Padding solution of the anilid of 2,3-oxynaphthoic acid.*

|                                                              | Light shades. | Dark shades. | 90 |
|--------------------------------------------------------------|---------------|--------------|----|
| Anilid of 2,3-oxynaphthoic acid                              | 60 grams      | 120 grams    |    |
| Caustic soda lye of 34° Baumé                                | 100 cc.       | 200 cc.      |    |
| Ricinoleate of soda or the sodium compound of Turkey red oil | 200 grams     | 300 grams    | 95 |
| Made up to                                                   | 10 liters     | 10 liters    |    |

The anilid of 2,3-oxynaphthoic acid is stirred with the caustic soda lye and the ricinoleate of soda or the sodium compound 100 of the Turkey red oil, then covered with hot water, boiled and made up to the desired quantity. The impregnation is best conducted at about 30-40° C.

*Diazo solution.*—300 grams of para-nitro-ortho-toluidin are stirred with 600 cc. of

hydrochloric acid of 20° Baumé and dissolved in 2000 cc. of boiling water; to the cooled solution are added 1500 grams of ice, and 156 grams of sodium nitrite dissolved in 500 grams of water are allowed to run in slowly in a thin stream, while stirring continually, and the whole is made up with cold water to 10 liters.

*Dye-bath.*—10 liters of the above described diazo solution are filtered through calico and mixed with 10 liters of cold water, and shortly before dyeing 1600 cc. of a solution of sodium acetate (1:1), are added.

For a subsequent treatment the following solution may be made:—10 liters of diazo solution are mixed with 5 liters of cold water, and 1600 cc. of a solution of sodium acetate (1:1) are added.

After dyeing, the yarn is well wrung out, well washed and twice soaped at a temperature of 70–80° C.

In this manner scarlet red tints of very great brightness and excellent fastness, are obtained.

*Example II. Production of the dyestuff, obtained by combining diazotized ortho-anisidin with the anilid of 2,3-oxynaphthoic acid, on cotton-yarn.*

The cotton yarn is impregnated with a solution of the anilid of 2,3-oxynaphthoic acid as prescribed in Example I and dyed in the same manner in a dye-bath of the following constitution:—

*Diazo solution.*—500 grams of ortho-anisidin are mixed with 1200 cc. of hydrochloric acid of 20° Baumé and dissolved in 1600 cc. of boiling water, to the cold solution are added 4000 grams of ice and a solution of 310 grams of sodium nitrite in 1000 grams of water is allowed to run in slowly, while stirring continually and the whole is made up to 10 liters.

*Dye-bath.*—5 liters of the above described diazo solution are mixed with 14 liters of cold water and shortly before dyeing 1200 cc. of a solution of sodium acetate (1:1) are added.

For a subsequent treatment the following solution is made:—5 liters of the diazo solution are mixed with 7 liters of cold water and 1200 cc. of a solution of sodium acetate (1:1) are added.

In this manner a beautiful deep cherry-red color, also of good fastness, is obtained.

*Example III. Production of the dyestuff, obtained by combining diazotized  $\alpha$ -naphthylamin with the anilid of 2,3-oxynaphthoic acid, on cops.*

The material is impregnated in the usual apparatus for dyeing cops, with the following:—

*Padding solution of the anilid of 2,3-oxynaphthoic acid.*—120 grams of anilid of

2,3-oxynaphthoic acid, 200 cc. of caustic soda lye of 34° Baumé and 250 grams of Turkey red oil are made up to 10 liters. The material is well drained, then subjected to the following dyebath, and well washed.

*Diazo solution.*—578 grams of  $\alpha$ -naphthylamin are stirred with 1040 cc. of hydrochloric acid of 20° Baumé and dissolved in 4000 cc. of boiling water. To the cold solution are added 2000 grams of ice and a solution of 320 grams of sodium nitrite in 1000 cc. of water is allowed to run in slowly while stirring and the whole is made up to 10 liters.

*Dye-bath.*—14 liters of ice-water are mixed with 5 liters of the above described diazo solution and shortly before dyeing 1200 cc. of a solution of sodium acetate (1:1) are added.

For a subsequent treatment the following solution is made: 7 liters of diazo solution are mixed with 5 liters of cold water and 1200 cc. of a solution of sodium acetate (1:1) are added.

By this combination dark red shades of good fastness are obtained.

*Example IV. Production of the dyestuff, obtained by combining tetrazotized ortho-tolidin with the anilid of 2,3-oxynaphthoic acid, on cotton yarn.*

The cotton-yarn is impregnated with a solution of the anilid of 2,3-oxynaphthoic acid as prescribed in Example I and dyed in the same manner in a dyebath of the following constitution:

*Diazo solution.*—420 grams of ortho-tolidin are mixed with 420 cc. of hydrochloric acid of 20° Baumé and dissolved in 3000 cc. of boiling water, to the cold solution are added 4000 grams of ice and 600 grams of hydrochloric acid of 20° Baumé. Then a solution of 310 grams of sodium nitrite in 1000 grams of water is allowed to run in slowly, while stirring continually and the whole is made up to 10 liters.

*Dye-bath.*—10 liters of the above described diazo solution are mixed with 8 liters of water and shortly before dyeing 1600 cc. of a solution of sodium acetate (1:1) are added.

For a subsequent treatment the following solution is made:—10 liters of the diazo solution are mixed with 4 liters of cold water and 1600 cc. of a solution of sodium acetate (1:1) are added.

By this process very dark deep reddish blue shades of good fastness are obtained.

*Example V. Production of the dyestuff, obtained by combining tetrazotized  $\beta$ -naphthylamin with the anilid of 2,3-oxynaphthoic acid, on cotton yarn.*

The cotton yarn is impregnated with the following:

*Padding solution of the anilid of 2,3-oxy-naphthoic acid.*

|                                       | Light blue.     | Medium blue.    | Dark blue. |
|---------------------------------------|-----------------|-----------------|------------|
| 5                                     |                 |                 |            |
| Anilid of 2,3-oxy-naphthoic acid..... | 60 grams .....  | 120 grams ..... | 240 grams. |
| Caustic soda lye of 84° Baumé.....    | 80 cc.....      | 160 cc.....     | 270 cc.    |
| Ricinoleate of soda.....              | 150 grams ..... | 300 grams ..... | 500 grams. |
| Made up to.....                       | 10 liters ..... | 10 liters ..... | 10 liters. |

- 10 Then it is dyed in the following dye-bath:  
*Diazo solution.*—240 grams dianisidin-base are dissolved in 210 grams hydrochloric acid of 20° Baumé and 2500 grams boiling water; to the cooled solution are added 2000 grams ice and 150 grams hydrochloric acid of 20° Baumé and then 160 grams sodium nitrite dissolved in 500 grams water are allowed to run in slowly in a thin stream, while stirring continually. The whole is made up to 10 liters.

*Dye-bath.*

|                                           | Light blue.    | Medium blue.    | Dark blue. |
|-------------------------------------------|----------------|-----------------|------------|
| 25                                        |                |                 |            |
| Diazo solution .....                      | 600 cc.....    | 1250 cc.....    | 2500 cc.   |
| Solution of cupric chlorid 40° Baumé..... | 100 cc.....    | 200 cc.....     | 300 cc.    |
| Solution of chromic acid 1 : 10.....      | 25 cc.....     | 50 cc.....      | 100 cc.    |
| Crystallized sodium acetate.....          | 100 grams..... | 150 grams.....  | 250 grams. |
| Made up to.....                           | 10 liters..... | 10 liters ..... | 10 liters. |

- 30 After dyeing, the yarn is well washed and twice soaped at a temperature of 70–80° C.  
35 To obtain a more reddish blue shade and to increase the fastness to rubbing a subsequent

treatment with a hot solution of 5 grams of copper sulfate per liter is advisable.

In this manner very powerful and fast blue shades are obtained.

In the same manner the process can be made with other diazo compounds and other arylamids of 2,3-oxy-naphthoic acid.

The anilid of 2,3-oxy-naphthoic acid can be substituted for example by the toluids, 45 the chloroanilids, the nitroanilids of 2,3-oxy-naphthoic acid. Instead of para-nitro-ortho-toluidin—see Example I—para-nitroanilin, ortho-nitroanilin, meta-nitroanilin, meta-nitro-para-toluidin, para-chloro-ortho-nitroanilin, meta-nitro-ortho-anisidin, para-nitro-ortho-anisidin can be employed.

Now what we claim and desire to be secured by Letters Patent is the following:

In the art of producing ice-colors on cotton the improvement consisting in treating cotton goods, which have been impregnated with a solution of an arylamid of 2,3-oxy-naphthoic acid, but have not been dried, with a non-sulfonated diazo compound.

In testimony, that we claim the foregoing as our invention, we have signed our names in presence of two witnesses this second day of October 1918.

ADOLF WINTHER.

AUGUST LEOPOLD LASKA.

ARTHUR ZITSCHER.

FELIX KUNERT.

EDWIN ACKER.

Witnesses:

JEAN GRUND,

CARL GRUND.